

March 30, 1937.

E. J. KAUFFMAN

2,075,039

APPARATUS AND METHOD FOR CONTROLLING FREEZING OF INGOTS

Filed Nov. 16, 1934

4 Sheets-Sheet 1



Fig. 1.



Fig. 2.



Fig. 5.



Fig. 3.



Fig. 4. INVENTOR.  
Edmund J. Kauffman

BY

Ramsey & Kent  
his ATTORNEYS

March 30, 1937.

E. J. KAUFFMAN

2,075,039

APPARATUS AND METHOD FOR CONTROLLING FREEZING OF INGOTS

Filed Nov. 16, 1934

4 Sheets-Sheet 2



*Fig. 6.*

*Fig. 11.*



*Fig. 10.*

*Fig. 12.*

INVENTOR.

*Edmund J. Kauffman*  
BY  
*Ramsey & Kent*  
his ATTORNEYS

March 30, 1937.

E. J. KAUFFMAN

2,075,039

APPARATUS AND METHOD FOR CONTROLLING FREEZING OF INGOTS

Filed Nov. 16, 1934

4 Sheets-Sheet 3



*Fig. 7*

*Fig. 8.*  
INVENTOR.  
Edmund J. Kauffman  
BY  
Ranney & Kent  
his ATTORNEYS

March 30, 1937.

E. J. KAUFFMAN

2,075,039

APPARATUS AND METHOD FOR CONTROLLING FREEZING OF INGOTS

Filed Nov. 16, 1934

4 Sheets-Sheet 4



*Fig. 13.*



*Fig. 14.*



*Fig. 15.*

INVENTOR.  
*Edmund J. Kauffman*  
BY  
*Ramsey & Kent*  
his ATTORNEYS

## UNITED STATES PATENT OFFICE

2,075,039

## APPARATUS AND METHOD FOR CONTROLLING FREEZING OF INGOTS

Edmund J. Kauffman, Girard, Ohio, assignor to  
 Valley Mould & Iron Corporation, Hubbard,  
 Ohio, a corporation of New York

Application November 16, 1934, Serial No. 753,297

10 Claims. (CL 22—200)

The present invention relates primarily to metallurgy and more specifically to an apparatus and method of controlling the freezing of ingots. It is further specifically related to the controlling of the freezing of steel ingots in molds equipped with hot tops.

Ingots formed in molds equipped with hot tops, and more especially molds of the big-end-up type, are with few exceptions, made from fully de-oxdized or "killed" steel. Such ingots are subject to internal cracks or ruptures extending longitudinally of the ingot and are known to those skilled in the art as "internal columnar dendritic ruptures", or more colloquially known as "internal point cracks". The lower carbon nickel steels some of the higher carbon plain steels, and in general, steels used for gears and high grade forgings are particularly subject to this very serious and dangerous defect.

The defects specified are brought about by permitting the ingot to stand in the mold until it is substantially frozen. During the freezing of the steel, the metal of the ingot shrinks as it solidifies, withdrawing the surface of the ingot from the matrix side walls of the molds. In substantially all cases, the frozen ingot tips to one side, thereby leaving one side of the ingot in contact with the mold and the other side of the ingot spaced apart from the matrix walls of the mold. This results in an uneven cooling of the ingot which develops these serious cracks, usually comprising hidden flaws, which result in very serious and dangerous weaknesses in the finished products. Attempts are made to avoid the flaws specified by removing the ingot from the mold before it is completely solidified. In order to do this, it becomes necessary to remove the hot top. As soon as the hot top is removed, the hot metal in the upper end of the ingot quickly freezes and the result is serious piping and porosity within the interior of the ingot as well as non-uniform freezing due to air drafts and other factors. It, therefore, is apparent that the metallurgist in attempting to cure one evil develops another which likewise produces serious defects.

The present invention overcomes the difficulties above specified and obviates the defects in the ingot by the method of longitudinally sliding the ingot within the mold, thereby obtaining additional air space between the ingot and the mold due to the taper of the matrix of the mold, maintaining the ingot centrally located within the mold to provide the air space between the ingot and the mold substantially uniform, then retaining the ingot within the mold until the ingot is substantially frozen, and with a hot top in position on the ingot during the period the ingot remains within the mold.

The preferred apparatus comprising one embodiment of the present invention is mechanism

such as a thrust plug to lift the ingot, and mechanism to guide and hold the ingot centrally located within the mold. The guide, which preferably is for the upper end of the ingot, may cooperate with the hot top or may cooperate directly with the ingot.

The disclosure herewith is illustrative of the present invention, and, therefore, is not to be considered in the limiting sense since it is realized that the present invention may be carried out with, and embodied in, structures other than those specifically disclosed herewith.

Fig. 1 is a cross-sectional view on line A—A of Fig. 5, illustrating the relation of the mold and the metal within the mold shortly after the pouring is completed.

Fig. 2 is a section on line A—A of Fig. 5 showing the relation of the metal within the mold and the mold during a later period in the stage of freezing.

Fig. 3 is a section on line A—A of Fig. 5 illustrating a still further stage in the freezing of the metal in the mold.

Fig. 4 is a cross-section of an ingot on the line A—A of Fig. 5 showing the ingot substantially frozen and illustrating the formation of internal columnar dendritic ruptures at the corners of the ingot adjacent sides of the ingot which have been in contact with the mold.

Fig. 5 is a vertical cross-section through the mold and ingot with the cross-section being taken through the ingot on line B—B of Fig. 4.

Fig. 6 is a section through a big-end-up ingot to which applicant's invention has been applied. This section is on the same plane as section A—A and corresponds to the stage of freezing of the defective ingot illustrated in Fig. 3.

Fig. 7 illustrates a vertical cross-section through a mold showing the initial stage of freezing of the metal in the mold with the set-up including a refractory type hot top telescoped into the upper end of the mold.

Fig. 8 illustrates applicant's method of control as applied to the ingot illustrated in the mold in Fig. 7.

Fig. 9 is a plan view of the construction illustrated in Fig. 8.

Fig. 10 is a vertical section through the upper end of a big-end-up mold equipped with apparatus embodying the present invention comprising guide pins for guiding the vertical movement of the hot top.

Fig. 11 illustrates a vertical sectional view through the upper end of a hot top guided by a suitable flange.

Fig. 12 illustrates a vertical section through the upper end of a hot top of the type illustrated in Fig. 7 showing a guide sleeve for the upper end of the ingot, which sleeve is mounted on the mold.

Fig. 13 illustrates a cross-section of a modifi-

cation of the embodiment illustrated in Fig. 12 comprising a hot top having a supporting shell guided by centering guide arms mounted on the mold.

5 Fig. 14 illustrates a vertical cross-section of an ingot mold and ingot with the ingot mold provided with an inward taper adjacent the upper end thereof to guide and center the raised ingot within the mold.

10 Fig. 15 illustrates a vertical cross-section of the upper end of an ingot mold with a hot top construction mounted within a shield of refractory material supported in a shell provided with guides cooperating with the shell of the hot top.

15 It is to be understood that the mold constructions illustrated in Figs. 10, 11, 12, 13 and 15 have the same lower constructions as are illustrated in Figs. 7, 8, and 14 and that the ingot has been raised in the Figs. 10, 11, 12, 13, and 15.

20 Fig. 1 illustrates a cross-section on line A—A of Fig. 5 and shows an ingot mold 1 having an eight sided fluted matrix. This type of contour is frequently used in the art to produce steel ingots that are most subject to internal point cracks. The molten metal which will form the ingot 2 within the mold is illustrated as beginning to form a skin 4 of dendritic columnar crystals with the skin 4 in contact with the walls of the matrix. At the stage of the freezing illustrated in Fig. 1, the skin 4 on the ingot is very thin and hot, and, therefore, is elastic and the metallo-static pressure of the molten interior metal forces this initial skin firmly against the matrix mold walls at all points. The crystals 25 at this stage represent a very thin chill zone of very fine crystals. As the freezing continues, these crystals build up in the form of acicular crystals comprising dendritic crystalline formation having their long axes substantially perpendicular to the mold matrix surfaces.

30 Fig. 2 illustrates a later stage of the freezing of the ingot taken on the same horizontal plane as Fig. 1. In Fig. 2, the corners 5 of the ingot have pulled away from the recesses 6 of the mold leaving the side walls 7 of the ingot in contact with the side walls 8 of the mold. This pulling away action at the corners may be due to several causes, one of which may be the tendency of the shrinking ingot to cause the circumference thereof to approach a more nearly circular form. As soon as the ingot breaks contact with the recesses 6 of the matrix of the mold, the direct conduction of heat at these zones is interrupted, thus causing the salients or 35 corners on the ingot to increase in temperature due to heat from the molten interior, while the zones 1, which are retained in contact with the mold wall, are being rapidly cooled as the heat of these side zones is absorbed by the mold. This 40 interrupts the growth of the acicular dendritic crystals at the corners while this type of crystals continues to grow on the sides of the ingot in contact with the mold.

45 Fig. 3 illustrates a further stage in the freezing of the ingot at which the circumference of the ingot has been substantially reduced in size and the ingot has tipped to one side of the matrix, so that while the sides 7 of the ingot are in contact with the matrix side walls 8 the sides 9 of the ingot 50 are out of contact with the side walls 10 of the mold and an air space extends around four of the sides of the eight sided ingot. As the ingot continues to freeze, the result is that the growth of the acicular dendritic crystals on the four side 55 walls 7 greatly predominate over the growth of

these crystals on the other four side walls 9. Consequently, the freezing of the ingot and the crystallization thereof is unbalanced. This causes the formation of the internal point cracks 11 illustrated in Figs. 4 and 5. These cracks ordinarily do not come entirely to the surface of the ingot although in exaggerated cases, that may happen. One reason for these internal cracks occurring at the corners and beneath the initial skin appears to be that the outer skin is usually of sufficient strength to resist shrinkage forces without cracking while the metal between the outer skin and the liquid core is weak. Since the shrinkage occurs most rapidly on the side faces, because they are in contact with the mold while the corners are out of contact, the metal of the ingot side walls inside the initial skin shrinks, and as it shrinks the crystals tend to swing like stalks of wheat toward the middle of the side walls. This tendency becomes so great and the hot metal inside the initial skin is of such low strength that voids occur where opposing shrinkage forces meet, thereby separating the crystals being pulled in one direction from adjacent crystals being pulled in the other direction. This occurs adjacent the corners which are not in direct contact with the mold. The result is longitudinal voids in the ingot comprising internal columnar dendritic ruptures such as are illustrated in Figs. 4 and 5.

30 It has been found by experiment that where the length of the acicular dendritic crystals in the middle of the side walls greatly exceeds the length of the dendritic crystals in the salients or corners, internal columnar dendritic ruptures are likely to appear. Referring to Fig. 3 and assuming the length of the dendritic crystals in the side wall out of the contact with the mold be represented by the character T and that the dendritic crystals of the adjacent corner be represented by the character K. If the ratio of T divided by K is not greater than the empirical number 2.25, the ruptures do not occur. On the opposite sides of the ingot illustrated in Fig. 3, where the ratio of T—1 divided by K—1, exceeds 2.25, ruptures do occur.

40 Where the ingot is held with its axis coincident with the axis of the mold so that the ingot cannot tip sidewise in the mold, then a condition is produced which is illustrated in Fig. 6, wherein a continuous air space, entirely around and substantially uniform, is provided between the matrix side walls and the ingot. This prevents unbalanced chilling of the ingot and tends to limit or stop the growth of the acicular dendritic crystals so that the molten interior of the ingot may solidify in 45 the form of axial crystals which do not produce the internal columnar dendritic ruptures.

50 Fig. 7 illustrates the initial freezing of an ingot in a big-end-up mold shortly after complete pouring and wherein the initial skin has just begun to shrink. At this stage of freezing, the lower portion and the upper portion of the ingot have substantially receded from the mold walls, whereas the middle portion indicated at 12—14 in Fig. 7 is still substantially in contact. In other words, 55 the ingot is somewhat barrel-shaped. This is due to the fact that the lower portion being poured first has had a longer time to cool and acquired strength, and the upper portion being under less metallo-static head already has sufficient strength to resist internal forces and to recede slightly from the mold walls. The middle zone has not sufficient strength to resist these internal forces and remains longer in contact with the matrix walls than other portions of the ingot. Very shortly 60

after this stage is reached, the ingot may be raised in the mold without rupture of the mold skin.

Fig. 8 illustrates the ingot 2 as being slid longitudinally in the mold 1 by means of a bottom plug 15 which contacts with the stool 16. The upper portion of this plug 15 is tapering while the lower part is cylindrical to be guided by the opening in the mold. This stool 16 is provided with an opening 17 to receive the plug 15 at the time when the metal is poured as shown in Fig. 7. After the initial ingot skin has reached the stage sufficient to support the molten metal within the ingot, the mold is raised by lugs commonly provided on ingot molds, shifted slightly on the stool 16 and set down with the end of the plug 15 contacting with the surface of the stool so that the weight of the mold 1 causes it to drop away from the ingot. As soon as this occurs, spacing plates 18 may be inserted between the mold and the ingot, as illustrated in Figs. 8 and 9, to hold the ingot centrally positioned within the mold and with a substantially uniform air space 19 around the ingot. In the construction illustrated in Fig. 8, the upper end of the ingot is unprotected. While the present invention may be carried out in this manner, it is preferable that the upper end of the ingot be protected against air cooling.

Fig. 9 is a plan view of the structure illustrated in Fig. 8, and shows a substantially rectangular contour mold provided with lifting lugs 20 common in the art. It is to be understood that the present invention is not confined to any particular cross-section contour of the matrix of a mold. The contour chosen in Figs. 1 to 6 more fully illustrates the invention, as a contour in common use and one wherein the difficulties here overcome most frequently occur. These same difficulties, however, occur with any mold in which the ingot tips sidewise to contact with the mold walls on one side only and thereby be unequally chilled.

Fig. 10 illustrates the present invention being carried out by an apparatus comprising a hot top having a metallic casing 21 carrying a refractory lining 22 and with guide pins 24 slideably movable through bearings 25 in the top of the mold. A shield may be provided around the lower portion of the hot top and is of sufficient length to protect the upper end of the ingot against air cooling when the ingot has been pushed upwardly to extend slightly from the mold. The pins 24 perform the double function of centering the hot top shell 21 over the mold and also of providing guides which hold the upper end of the ingot centrally located relative to the mold matrix when the ingot has been moved longitudinally in the mold.

Fig. 11 illustrates a modification of a construction shown in Fig. 10 and wherein a guide shield is provided to center the hot top on the mold and to guide the hot top when the ingot is lifted in the mold. Either member, i.e., the mold or hot top, may carry the shield 26 so long as it is held in place to perform the function of guiding the relative movement of these parts to maintain the ingot centrally located when the ingot is lifted.

Fig. 12 illustrates a section through the upper end of the mold and hot top wherein the hot top is similar to that illustrated in Fig. 7 and is guided in its upward movement by a flange comprising a guide shield 28 for the ingot when it is lifted. This flange guide member 28 is preferably carried by the mold 1 and may be secured there-

to by key pins 27 passing through the edge of the flange 28 and lugs 29 provided on the mold 1.

Fig. 13 illustrates a refractory lined hot top having a metallic shell provided with a cylindrical portion 30 adapted to cooperate with guide fingers 31 secured to the upper end of the mold by the key pins 27.

Fig. 14 illustrates a mold set-up in which the major portion of the matrix 32 has an upward and outward taper, whereas the matrix from the point 34 to the mouth of the mold is provided with an inward taper 35 of such amount as to contact with the upper end of the ingot when it is raised to position the same centrally within the mold 1. In this construction, the hot top 36 telescopes within the mold so that the bottom of the hot top during pouring is located substantially at the point 34 or slightly below in the matrix of the mold.

Fig. 15 illustrates a further modification of the present invention in which a flange 36 is secured to the mold body by key pins 27 and the interior face of the flange is lined with refractory material 37 to act as a heat insulator for the upper end of the ingot 2 when the same is lifted to provide the uniform air space 19 around the ingot. This flange is provided with guide lugs 38 which cooperate with the cylindrical portion 30 on the hot top to guide the same.

It is to be understood that if Figs. 10, 11, 12, 13, and 15 were completed, the lower portions of the figures would be identical with the full constructions illustrated in Figs. 8 and 14.

In order to give a specific example of the operation of the present invention, a specific mold and ingot will be analyzed. The type of contour illustrated in Figs. 1, 2, 3, and 6 will be chosen and it will be assumed that the mean diameter or mid section of the ingot on line A—A of Fig. 5 is 26 inches. The weight of a steel ingot poured not including the sink head portion is 10,050 pounds and the weight of the ingot plus the sink head is 12,100 pounds. Assume that the steel is to be .30% carbon or less with 3.50% nickel, which is a steel that is very sensitive to the development of these internal corner cracks. For this size mold, the rate of pouring of metal at normal pouring temperatures is not to exceed the rate of one gross ton per minute. After the pour is completed, the ingot should remain quietly in the mold with the hot top thereon for approximately one and three quarter hours. At the expiration of this time, the mold is lifted by lift rig 39 (Fig. 7) attached to a suitable overhead crane. The lift rig 39 engages the lugs 20 provided for this purpose and the mold when lifted is moved sufficiently to cause the centering and ejecting plug 15 to engage the top surface of the stool 16 when the mold is lowered, thereby causing the mold to drop away from the ingot or in other words, causing a relative longitudinal movement between the ingot and the mold. Preferably, the amount of the relative movement is substantially eight inches. The preferred taper of the mold is such as will provide substantially a one quarter inch space between the surface of the ingot and the matrix side walls of the mold for the movement specified. The air shield provided prevents air cooling the upper end of the ingot and the lifting of the ingot relatively to the mold has caused the upper end thereof to snugly fit within the hot top which has been accurately guided and held in its final position to substantially center the ingot in the manner specified. The ingot and mold are preferably retained in their telescoped relation for three or

four hours, after which the ingot may be stripped from the mold in the usual manner and thereafter treated in accordance with the specific procedure of the mill utilizing the present inventions by 5 removing the ingot to a suitable pit or to a re-heating furnace for direct forging or rolling as the case may be.

It is to be understood that for different sized molds and ingots the pouring speed and the time 10 the ingot remains in the mold are to be varied according to the teaching of the art well known to those skilled in the art.

An important feature of the invention is the maintenance of the uniform air space around the 15 ingot during the final stages of freezing of the ingot, and preferably until the dendritic crystals have substantially ceased to form in the ingot.

What I claim is:

1. In a device of the class described, a big-end- 20 up ingot mold, a hot top movably mounted on said mold, the hot top being of rigid construction which becomes attached to the ingot, means to cause a relative longitudinal bodily movement between said mold and a partially frozen ingot 25 therein, and means to positively guide said rigid hot top during said movement to retain the axis of said ingot substantially coincident with the axis of the matrix of said mold when said movement has occurred.

30 2. Apparatus for casting ingots and soaking them in the mold during the later stages of solidification, comprising: a big-end-up ingot mold; a hot top mounted movably on said mold to permit the hot top to remain in place on the ingot during 35 partial stripping of an ingot cast in said mold; means to partially strip the ingot, sufficiently to establish a heat insulating air space between the ingot and the mold, said construction maintaining said air space closed against the circulation 40 therethrough of substantial currents of cooling air; and means cooperating with the hot top to hold the hot top and ingot coaxial with the mold upon completion of said partial stripping.

3. Apparatus for casting ingots and soaking 45 them in the mold during the later stages of solidification, comprising: a big-end-up ingot mold; a hot top mounted movably on said mold to permit the hot top to remain in place on the ingot during partial stripping of an ingot cast in said mold; 50 means to partially strip the ingot, sufficiently to establish a heat insulating air space between the ingot and the mold, said construction maintaining said air space closed against the circulation therethrough of substantial currents of cooling 55 air; and means to hold the ingot coaxial with the mold upon completion of said partial stripping.

4. Apparatus for casting ingots and soaking them in the mold during the later stages of solidification, comprising: a big-end-up ingot mold; 60 a hot top mounted on said mold; means to partially strip an ingot cast in said mold, sufficiently to establish a heat insulating air space between the ingot and the mold, said construction maintaining said air space closed against the circulation therethrough of substantial currents of cooling air; and a telescopic connection between said 65 hot top and said mold, said connection permitting the hot top to remain on the ingot during said partial stripping and then maintaining the ingot coaxial with the mold.

5. Apparatus for casting ingots and soaking 70 them in the mold during the later stages of solidification, comprising: a big-end-up ingot mold;

means to partially strip an ingot cast in said mold, sufficiently to establish a heat insulating air space between the ingot and the mold, said construction maintaining said air space closed against the circulation therethrough of substantial currents of cooling air; and means to maintain the ingot coaxial with the mold after said partial stripping has been effected.

6. Apparatus for casting ingots and soaking 10 them in the mold during the later stages of solidification, comprising: a big-end-up ingot mold; a hot top mounted on said mold, free to be separated therefrom in an axial direction; means to partially strip an ingot cast in the mold, sufficiently to separate the hot top from the mold and establish a heat insulating air space between the ingot and the mold, said construction 15 maintaining said air space closed against the circulation therethrough of substantial currents of cooling air; and means to hold the ingot coaxial with the mold upon completion of said partial stripping and also shield the ingot from cooling currents in the zone between the mold and the hot top.

7. The method of controlling the freezing of 25 a steel ingot after it has been poured in a tapered ingot mold, which comprises: partially stripping the ingot, sufficiently to establish a heat insulating air space between the ingot and the mold; maintaining said air space substantially uniform about the periphery of the ingot, 30 heat insulating the upper end of the ingot, and preventing substantial circulation of cooling air through said space.

8. The method of controlling the freezing of 35 a steel ingot after it has been poured in a tapered ingot mold, which comprises: partially stripping the ingot when the sides of the ingot have frozen to a self-supporting thickness, the 40 partial stripping being sufficient to establish a heat insulating air space between the ingot and the mold; maintaining said air space substantially uniform about the periphery of the ingot, heat insulating the upper end of the ingot, and preventing substantial circulation of cooling air 45 through said space.

9. The method of controlling the freezing of 50 a steel ingot after it has been poured in a tapered ingot mold, which comprises: partially stripping the ingot, sufficiently to establish a heat insulating air space between the ingot and the mold while leaving the major portion of the ingot inside of the mold; preventing substantial circulation of cooling air through said space; heat insulating the upper end of the ingot; and maintaining the ingot coaxial with the mold in said 55 partially stripped position until dendritic crystals have substantially ceased to form in the ingot.

10. The method of controlling the freezing of 60 a steel ingot after it has been poured in a tapered ingot mold, which comprises: partially stripping the ingot, sufficiently to establish a heat insulating air space between the ingot and with a minor portion of the ingot projecting outside of the mold; preventing substantial circulation of cooling air through said space; protecting the projecting portion of the ingot from cooling currents of air; and maintaining the ingot coaxial with the mold in said partially stripped position until dendritic crystals have substantially ceased to form in the ingot.

EDMUND J. KAUFFMAN.